

## UNITED STATES PATENT OFFICE

2,276,233

DEODORIZATION AND REFINING OF  
TUNG OIL

Louis A. Gruenwald and Malcolm John Reider,  
New York, N. Y.; said Reider assignor to said  
Gruenwald

No Drawing. Application March 11, 1940,  
Serial No. 323,400

5 Claims. (Cl. 260—420)

The present invention relates to the deodorization of tung oil and it also in its more broader aspects relates to the refining of other types of oils.

Considerable difficulty has been experienced in deodorizing tung and similar unsaturated drying glyceride oils without disadvantageously affecting their drying properties because of the expense involved and the resultant decrease in quality of the oil.

As a general rule, these deodorization treatments require complicated and expensive apparatus and frequently they did not produce an oil which had satisfactory stability or which could be most desirably utilized with or without further processing in various textile procedures for either finishing or otherwise treating textile yarns or fabrics.

It is among the objects of the present invention to provide an improved process for the deodorization and refining of tung and other similar drying oils, which may be carried out by relatively inexpensive procedure without complicated apparatus or involved process steps, and which will produce a high grade deodorized oil having satisfactory stability characteristics and which will not have lost any of its initially desirable characteristics or qualities.

Still further objects and advantages will appear from the more detailed description set forth below, it being understood, however, that this more detailed description is given by way of illustration, since various changes therein may be made by those skilled in the art without departing from the scope and spirit of the invention.

In accomplishing the above objects it has been found most satisfactory to subject the tung oil to treatment with a compound or salt of a reducing sulphur acid in which the sulphur preferably has a valence of less than 6 and in which the sulphur acid preferably is combined with either an alkali metal or an alkali earth metal in the form of a salt.

This sulphite treatment may desirably be followed by a treatment with a relatively heavy metal salt, such as for example a lead salt.

It has been found that the refining and deodorization of the tung oil may be satisfactorily obtained when either of these treatments are used alone, and it is contemplated to include within this invention the treatment of the tung oil with sodium sulphite by itself or with a lead salt, such as for example lead acetate, sulphate, chloride or nitrate or even a lead salt of a reducing sulphur acid of the character above described.

Without limiting the invention, it has been

found that the sulphite treatment may be satisfactorily carried out as by the following procedure.

In a large vessel, such as an open pot equipped for heating the body of tung or other oil may be placed which is to be processed.

To this vessel is then added about  $\frac{1}{10}$  to 1% of sodium sulphite, preferably in the form of a dilute aqueous solution.

10 It has been found satisfactory for instance to employ 10% by weight of a 5% aqueous solution of the sodium sulphite or acid sulphite.

The mixture of the oil with the sulphite is then heated with rapid stirring to 110° C. and after this temperature is reached, the oil is diluted with a thinner and then filtered, utilizing a filter aid.

15 Where the sulphite treatment is to be followed by a further treatment with a lead salt or compound, the addition of the thinner may be omitted, and after filtering or decantation of the oil, the oil may be directly subjected to the lead treatment.

20 As an example of a lead treatment which may be carried out in a similar sort of an open pot equipped for heating, the oil may be placed and then there may be added to such oil from  $\frac{1}{10}$  to 1% of a lead compound which may, for example, consist of the acetate, the chloride, the sulphate, the nitrate or even the oxide.

25 The mixture is rapidly stirred and heated to 110° C. after which the oil may be diluted with a thinner, such as heavy naphtha and filtered with the aid of a vacuum and in the presence of a filter aid, such as infusorial earth.

30 35 These two procedures, as given above, are quite inexpensive, do not require expensive apparatus and give a good yield of oil, which is substantially odorless.

Although it is not certain what action takes place, it is found that with the sodium sulphite treatment there apparently is a removal of aldehyde and ketone compounds. Although the same result is obtained even where solid sodium sulphite or a solution of sodium sulphite is added in the cold, nevertheless it has been found most satisfactory to heat the sulphite in the oil up to between 80 to 130° C., and preferably between 90 and 150° C.

40 45 It is found most desirable to have the sulphite present in sufficient amounts so that sulphur dioxide will be evolved during the heating operation, such evolution of sulphur dioxide apparently improving the color and causing bleaching of the oil, as well as removing some of the odor.

50 55 The steaming of the oil during the heating

procedure from the small amount of water present in an aqueous solution of the sodium sulphite also appears to be quite advantageous.

In connection with the treatment of the oil with a solid or more preferably an aqueous solution of a heavy metal salt, such as lead acetate, it again is found most satisfactory to have an evolution of steam during the treating procedure and preferably while the temperature of the mixture is being elevated to between 80 to 180° C., and preferably between 90 and 150° C.

The evolution of the steam in the presence of the lead salt appears to be particularly satisfactory, in that unpleasant smelling substances, which are responsible for the odor, are apparently readily removed and it also appears that the free fatty acids not only are largely eliminated by this heavy treatment, but also the tendency for further formation thereof is greatly reduced.

The lead and similar heavy metal salts also appear to body the oil at the same time as the deodorization takes place, depending upon the length of time the treatment is continued and the temperature of the treatment.

The lead or other heavy metal salts, and to a lesser degree, the sulphite treatment, also appear to precipitate or remove albuminous and protein-like substances which are found in natural oils and which are found to be responsible for many of their objectionable characteristics.

Although tung oil is preferred, it has been found that other paint or saturated or unsaturated glyceride oils may also be deodorized by either step or both steps of the present invention.

Among the oils which may be suitably processed are China-wood oil, soya bean oil, linseed oil, sunflower seed oil, rice bran oil, olive oil, cotton seed oil, neat's-foot oil and various other fish, animal and vegetable oils.

Although both the lead salt and alkaline sulphite should be in water soluble form so that they may be emulsified in small quantities through the body of the oil, while the oil is being heated, insoluble compounds may also be employed.

The preferred lead compounds are, however, the lead acetate, formate or other organic acid salts and less preferably inorganic acid salts, such as lead nitrate.

Among the other heavy metals which may be used in place of or in lieu of the lead are iron,

mercury, cobalt, zinc, nickel, tungsten and tin.

The alkali metal sulphites or bi-sulphites are usually most preferred because they are water soluble, although the less water soluble calcium sulphite or bi-sulphite may also be utilized.

It is also less preferable to use the thio-sulphates, hydro-sulphites, polythionates as well as other salts of reducing sulphur acids, preferably, however, excluding the sulphide.

As many changes could be made in the features and details, and many apparently widely different embodiments of this invention could be made without departing from the scope thereof, it is intended that all matter contained in the above description shall be interpreted as illustrative and not in a limiting sense.

What is claimed is:

1. A process of deodorizing tung oil which comprises heating the tung oil first with a small quantity of an aqueous solution of a sodium sulphite dispersed throughout the body thereof and then with a small quantity of an aqueous solution of lead acetate.

2. A process of deodorizing tung oil which comprising heating the tung oil first with a small quantity of an aqueous solution of a sodium sulphite dispersed throughout the body thereof and then with a small quantity of an aqueous solution of lead acetate at an elevated temperature between 75 and 180° C.

3. A process for deodorizing tung oil which comprises heating the tung oil first with a small quantity of an aqueous solution of a sodium sulphite dispersed throughout the body thereof and then with a small quantity of an aqueous solution of lead acetate at an elevated temperature between 90 and 150° C. with agitation.

4. A process of deodorizing a tung oil which comprises mixing in the tung oil about 10% by weight of a 5% aqueous solution of sodium sulphite, heating with rapid stirring to 110° C., diluting the oil with naphtha and then filtering with infusorial earth.

5. A process of deodorizing tung oil which comprises emulsifying into the oil about 20% by weight of a 3% solution of lead acetate, heating the mixture with rapid stirring to 110° C., diluting with heavy naphtha as a thinner and then filtering with the aid of vacuum and infusorial earth.

LOUIS A. GRUENWALD.  
MALCOLM JOHN REIDER.